

J. S. SEAMAN, JR.  
ROLL.  
APPLICATION FILED FEB. 24, 1913.

1,071,810.

Patented Sept. 2, 1913.

FIG. 1.



J. Herbert Bradley  
H. B. Hayes

FIG. 2.



Joseph S. Seaman, Jr.  
by Dennis D. Wolcott  
Atty

# UNITED STATES PATENT OFFICE.

JOSEPH S. SEAMAN, JR., OF PITTSBURGH, PENNSYLVANIA.

## ROLL.

1,071,810.

Specification of Letters Patent.

Patented Sept. 2, 1913.

Application filed February 24, 1913. Serial No. 750,284.

*To all whom it may concern:*

Be it known that I, JOSEPH S. SEAMAN, Jr., residing at Pittsburgh, in the county of Allegheny and State of Pennsylvania, a citizen of the United States, have invented or discovered certain new and useful Improvements in Rolls, of which improvements the following is a specification.

The invention described herein relates to certain improvements in rolls for reducing ingots, blooms or billets to rails, beams, channels, of other sections, and has for its object a roll having incorporated in its collars during the casting of the roll, metal rings, which serve during such manufacture to effect a localized cooling of the molten metal, whereby the metal thus affected is rendered more dense.

The invention is hereinafter more fully described and claimed.

In the accompanying drawing forming a part of this specification, Figure 1 is a sectional view of a portion of my improved roll, and Fig. 2 is a sectional view showing my improved roll with grooves to form rail passes and a collared roll used in connection therewith.

It is customary in manufacturing grooved rolls to form during the casting of the rolls, grooves approximating in width and depth the dimensions desired in the finished roll. The roll is finished by cutting away the metal for a considerable depth along the side walls and bottoms of the preliminary grooves, as will be seen by a comparison of Figs. 1 and 2, the former showing the grooves formed in the casting operation and the latter showing the completed grooves. As is well known in the art the metal adjacent to the surfaces of a casting is more dense, and in chill castings very much harder than the metal at a greater depth. In finishing the rolls a considerable proportion of the more durable metal is cut away, and as the hardness and density due to chill-

ing does not extend to any considerable depth the chilled metal will be entirely removed in one or two returnings of the roll.

As fully described in an application for Letters Patent Serial No. 728,707, filed October 30, 1912, a greater depth of dense and chilled metal can be attained by causing a rapid reduction of the temperature not only of the metal forming the surfaces *a* of the sides and bottoms of the grooves 7 but also of the metal relatively remote from the surface metal. This internal cooling of the metal intermediate of the grooves 7 is effected by means of ring 10, which is preferably formed of the same kind of metal as the roll. The ring is arranged in proper position in the mold prior to the teeming of the molten metal, as fully described and claimed in the application referred to, and becomes incorporated in the body of metal 6 adjacent to the groove.

By properly proportioning the transverse dimensions of the rings the entire body of metal in the collars 6 will be rendered dense and by making the internal peripheries of the rings less than the periphery of the bottoms of the grooves, the inward and lateral extent of dense metal at the corners of the groove is greatly increased.

I claim herein as my invention:

1. A grooved roll, having a metal ring incorporated within the periphery of the collars or portions intermediate the grooves of the roll.

2. A grooved roll, having a metal ring incorporated therein adjacent to a groove, the inner periphery of the ring being less than the periphery of the roll at the bottom of the groove.

In testimony whereof, I have hereunto set my hand.

JOSEPH S. SEAMAN, Jr.

Witnesses:

ALICE A. TRILL,  
THOS. B. JOYCE.